

## 1

2,992,181  
PROCESS FOR PRODUCING A PETROLEUM  
BASE PITCH

Jack F. Renner, Calumet City, Ill., assignor to Sinclair  
Refining Company, New York, N.Y., a corporation of  
Maine

No Drawing. Filed Sept. 11, 1957, Ser. No. 683,224  
4 Claims. (Cl. 208—22)

This invention relates to a method of producing a 10 petroleum base pitch and more particularly to the production of a novel petroleum base pitch having physical characteristics more comparable to coal tar pitch than conventional petroleum asphalts and pitches.

With the development of new applications in recent 15 years for coal tar products there has consequently been created an increasing demand for salable coal tar pitch. However, most coal tar products plants in the United States are operated by steel companies and the pitch produced by the distillation of coal tar is utilized by these companies as fuel for their open hearth furnaces. Consequently, of the total volume of coal tar produced in the country only a very small percent is available as salable pitch. To meet the increasing demand for coal tar pitch attempts have been made to find a petroleum pitch comparable in all respects to coal tar pitch. Investigations have proved fruitless particularly in uncovering a petroleum pitch possessing the low needle penetration, low molten viscosity and high insolubility in benzene, naphtha and kerosene that characterizes the coal tar pitches.

It has now been found that a homogeneous petroleum base pitch that compares favorably with coal tar pitch may be produced by heating at a temperature of about 700° to about 1000° F., a feedstock composed of petroleum bottoms obtained from distilling a cracked oil produced by catalytic cracking processes. The employment of a high temperature from about 700° to about 1000° F. by itself is sufficient to produce the novel product of this invention. The effect of my novel process is the condensation or polymerization of aromatic material present in the feedstock to form higher molecular weight ring compounds that subsequently yield the pitch material of this invention. A petroleum pitch produced in this manner is found to exhibit physical characteristics markedly similar to those of coal tar pitch. In addition to high insolubility in benzene and petroleum naphtha, the pitch displays low penetration and low molten viscosity.

The feedstock of my invention must possess certain specific properties to yield a suitable pitch. An ideal feedstock would be composed substantially completely of aromatic ring compounds with little or very slight side chain substitution and a minimum molecular weight of 190. However, all commercially available feedstocks contain other components such as paraffins and non-reactive naphthenes and aromatics which tend to hinder pitch production and should for that reason be removed as a part of the processing sequence. If the latter materials are not removed, a non-homogeneous, valueless material is produced.

## 2

Feedstocks suitable for this process are characterized by the following approximate properties:

|                                                                                    |           |
|------------------------------------------------------------------------------------|-----------|
| Gravity, °API (ASTM D287-55)                                                       | 18.0 max. |
| Flash, °F. (ASTM D92-52)                                                           | 200 min.  |
| Average molecular weight                                                           | 190 min.  |
| Initial boiling point, °F.                                                         | 400 min.  |
| Chromatographic analysis:                                                          |           |
| Saturates, wt. percent                                                             | 50 max.   |
| Aromatics and polar compounds, wt. percent                                         | 50 min.   |
| Aromatic fraction—                                                                 |           |
| Average molecular weight                                                           | 190 min.  |
| Hazelwood ring analysis:                                                           |           |
| Average No. of rings per molecule                                                  | 3.5 min.  |
| Average No. of aromatic rings per molecule                                         | 3.0 min.  |
| Average No. of naphthenic rings per molecule structure                             | 1.0 max.  |
| Average No. of carbon atoms in aromatic ring structure                             | 13.0 min. |
| Average No. of carbon atoms in naphthenic rings and paraffin side chain structures | 5.0 max.  |

A petroleum refinery stock found to meet all of these requirements and yield a suitable pitch is the bottoms fraction obtained by the distillation of the cracked oil produced from the catalytic cracking of petroleum gas oils in the presence of catalyst such as the silica-alumina catalysts. In such processes the catalyst usually comprises about 65 to 95% silica and 5 to 35% alumina and is frequently employed in the fluidized state.

The cracked oil produced as a result of the fluid catalytic cracking process is then subjected to distillation at about 7 to 25 p.s.i. pressure to a maximum temperature of about 650 to 750° F. The residue or distillation bottoms obtained as a consequence of the above distillation process are transferred to a slurry settler for removal of catalyst and the resultant oil has been found to be a suitable refinery stock for the production of my novel petroleum base pitch. This petroleum bottoms fraction will be hereafter referred to as fluid unit clarified oil and the novel petroleum base pitch produced as clarified oil pitch. Although the present invention will be described with reference to the employment of fluid cracking unit clarified oil as the suitable feedstock, any petroleum feedstock meeting the property requirements set forth above may be used. Typical tests on satisfactory fluid unit clarified oils are shown below:

|                                                        | Tests on<br>Clarified<br>oil |
|--------------------------------------------------------|------------------------------|
| Gravity, °API (ASTM D287-55)                           | 4.5-12.5                     |
| Flash, °F. (ASTM D92-52)                               | 375-315                      |
| Fire, °F. (ASTM D92-52)                                | 450-420                      |
| Viscosity at 210° F., SSU (ASTM D88-53)                | 50-40                        |
| Aniline point, °C. (ASTM D611-55T)                     | 45-70                        |
| Molecular weight                                       | 280-330                      |
| Boiling range (90% distilled), °F.                     | 500-1000                     |
| Chromatographic analysis:                              |                              |
| Paraffins, wt. percent                                 | 23.0-38.0                    |
| Polar compounds, wt. percent                           | 2.0-2.0                      |
| Aromatics, wt. percent                                 | 75.0-80.0                    |
| Tests on aromatic fraction—                            |                              |
| Refractive index, 20/D                                 | 1.68-1.66                    |
| Density, 20/4° C.                                      | 1.12-1.09                    |
| Molecular weight                                       | 250-280                      |
| Hazelwood ring analysis:                               |                              |
| Average No. of rings per molecule                      | 4.4-4.2                      |
| Average No. of aromatic rings per molecule             | 3.7-3.6                      |
| Average No. of carbon atoms per molecule               | 20.8-19.0                    |
| Average No. of carbon atoms in ring structure          | 19.6-18.2                    |
| Average No. of carbon atoms in aromatic ring structure | 16.8-16.2                    |

Chromatographic analyses of various fluid unit clarified oil feedstocks show them as characterized by an aromatic content ranging from 50 to 75 weight percent of

these feedstocks; best yields being obtained from those possessing the highest aromatic content. The aromatic content of the clarified oils has been found to be dependent to some degree on fluid unit conversion levels (yield of 400 E.P. gasoline). For example, at 78.5% conversion pitch yield from the resultant clarified oil is 59.0%; whereas at 60% conversion yield is 45.0%. Generally speaking, the cracking unit must be operated at a minimum 50% conversion (50% yield of 400 E.P. gasoline) to yield a clarified oil that is an economical feedstock for my process.

Although a large variation is found in the aromatic content of the many fluid unit clarified oils, ring analyses of the aromatic fractions from both the clarified oils and their respective distillation cuts indicate very slight differences in composition. The average molecular structure by Hazelwood Ring Analyses, Analytical Chemistry, 26, 1073 (1954), of the aromatic fractions from clarified oils has been found to contain about 3.5 to 3.7 aromatic rings, 0.4 to 0.7 naphthenic ring, and 0.5 to 1.3 carbon atoms attached to the ring structure. Thus, the aromatic fractions are characterized as containing condensed ring molecules with slight side chain substitutions.

In carrying out the present invention a clarified oil meeting the property requirements set forth above is subjected to temperatures of about 700 to 1000° F., preferably about 750 to 800° F., for a period of at least about 10 hours. No particular advantage has been associated with heating time over about 50 hours but longer periods could be employed. Preferably, the heating time is about 10 to 20 hours. During this heating period substantially all of the non-reactive or unreactive wax-oil components in the clarified oil are removed as an overhead product. A petroleum base pitch is formed which exhibits low solubility in petroleum solvents, low molten viscosity and low needle penetration at 77° F. Although the majority of the undesirable unreacted material is taken overhead by virtue of the high processing temperatures, supplemental means such as steam stripping, vacuum distillation or solvent deoiling can be used to remove additional unreacted material.

The following example will further illustrate my invention, but it is not to be considered limiting.

#### EXAMPLE

1400 grams of fluid unit clarified oil possessing the physical properties described above was charged to an open kettle and heated for 30 hours at 750-800° F. A pitch yield of 50.9 weight percent was obtained. Tests on the resultant pitch and overhead oil are shown below:

|                                        |        |
|----------------------------------------|--------|
| Tests on clarified oil pitch:          |        |
| Specific gravity, 77°/77° F.           | 1.1490 |
| Softening point (R. & B.), ° F.        | 204    |
| Needle penetration at 77° F.           | 0      |
| Viscosity at 350° F., SFS              | 105    |
| Sulfur, wt. percent                    | 91.9   |
| Insolubles in 80° naphtha, wt. percent | 40.1   |
| Insolubles in benzene, wt. percent     | 26.1   |
| Gravity, ° API                         | 38.6   |
| Viscosity at 100° F., SFS              |        |

As shown in Table I below, there is a marked similarity between coal tar pitch and the clarified oil pitch produced by the process of my invention.

Table I

#### COMPARISON OF THE PHYSICAL PROPERTIES OF CLARIFIED OIL PITCH, COAL TAR PITCH AND BLOWN ASPHALT

|                                        | Clarified Oil Pitch | Coal Tar Pitch | Blown Asphalt |
|----------------------------------------|---------------------|----------------|---------------|
| Specific gravity, 77° F./77° F.        | 1.1490              | 1.1695         | 1.0190        |
| Softening point (R. & B.), ° F.        | 204                 | 187            | 178           |
| Needle penetration at 77° F.           | 0                   | 0              | 26            |
| Needle penetration at 115° F.          | 3                   | 2              | 49            |
| Needle penetration at 140° F.          | 4                   | .37            |               |
| Viscosity at 300° F., SFS              |                     | 164.9          |               |
| Viscosity at 350° F., SFS              | 105                 | 34             | 199.6         |
| Insolubles in benzene, wt. percent     | 40.1                | 36.9           | 0.4           |
| Insolubles in 80° naphtha, wt. Percent | 91.9                | 94.5           | 33.0          |

The pitch yielded by my invention exhibits high insolubility in petroleum fractions, vegetable oils and aromatic solvents as compared to normal petroleum asphalts and pitches. The pitch gives about a 5% maximum overhead when distilled to 640° F. and preferably this is about 1%. These physical characteristics make it particularly suitable for use as a fuel resistant airport paving cement, a fuel resistant pipe coating enamel, a fiber pipe impregnant, a saturant for weatherboard, siding and insulating board, a rubber plasticizer, a sandmold binder, a molding compound, an additive for paints and a waterproofing compound. The clarified oil pitch of the invention is not limited to the above applications but may also be employed anywhere coal tar pitch has been used or wherever its novel physical properties offer advantageous results.

I claim:

1. A process for producing a petroleum base pitch which comprises heating for about 10 to 50 hours at a temperature of about 700 to 1000° F. a petroleum bottoms feedstock obtained from the distillation of the cracked oil produced by the catalytic cracking of petroleum gas oils, said feedstock having the following approximate properties:

|                                                                                    |           |
|------------------------------------------------------------------------------------|-----------|
| Gravity, ° API (ASTM D287-55)                                                      | 18.0 max. |
| Flash, ° F. (ASTM D92-52)                                                          | 200 min.  |
| Average molecular weight                                                           | 190 min.  |
| Initial boiling point, ° F.                                                        | 400 min.  |
| Chromatographic analysis:                                                          |           |
| Saturates, wt. percent                                                             | 50 max.   |
| Aromatics and polar compounds, wt. percent                                         | 50 min.   |
| Aromatic fraction:                                                                 |           |
| Average molecular weight                                                           | 190 min.  |
| Hazelwood ring analysis:                                                           |           |
| Average No. of rings per molecule                                                  | 3.5 min.  |
| Average No. of aromatic rings per molecule                                         | 3.0 min.  |
| Average No. of naphthenic rings per molecule                                       | 1.0 max.  |
| Average No. of carbon atoms in aromatic ring structure                             | 13.0 min. |
| Average No. of carbon atoms in naphthenic rings and paraffin side chain structures | 5.0 max.  |

and removing by distillation the unreacted naphthene and aromatic components from the pitch obtained to produce a homogeneous petroleum-base pitch giving a maximum overhead of about 5% when distilled to 640° F.

2. The process of claim 1 wherein the petroleum bottoms feedstock is obtained from the distillation of the cracked oil produced by the fluid catalytic cracking of petroleum gas oil.

3. The process of claim 1 wherein the heating of the feedstock is conducted at a temperature of about 750 to 800° F.

4. A petroleum base pitch produced by the method of claim 1.

#### References Cited in the file of this patent

#### UNITED STATES PATENTS

|           |                 |                |
|-----------|-----------------|----------------|
| 2,029,288 | Bray            | Feb. 4, 1936   |
| 2,626,892 | McCulley et al. | Jan. 27, 1953  |
| 2,658,857 | Roediger        | Nov. 10, 1953  |
| 2,752,290 | Beattie         | June 26, 1956  |
| 2,763,602 | Cole            | Sept. 18, 1956 |
| 2,764,527 | Steele et al.   | Sept. 25, 1956 |
| 2,796,388 | Beuther et al.  | June 18, 1957  |